

Dec. 13, 1966

V. PETROVICH

3,290,742

GRAIN REFINING PROCESS

Filed Feb. 6, 1964

Segment 1   Segment 2   Segment 3   Segment 4



Fig. 1

Segment 1   Segment 2   Segment 3   Segment 4



Fig. 2

Chilled surface  
of casting

INVENTOR.  
Vladimir Petrovich

BY

Griswold & Gurdick  
ATTORNEY

1

3,290,742  
GRAIN REFINING PROCESS

Vladimir Petrovich, Midland, Mich., assignor to The Dow Chemical Company, Midland, Mich., a corporation of Delaware

Filed Feb. 6, 1964, Ser. No. 343,067  
9 Claims. (Cl. 22—200.1)

This invention relates to grain refining and more particularly relates to a novel method of grain refining a magnesium-base alloy containing zinc and misch metal.

When casting magnesium alloys containing up to 1.0 percent of rare earth metals and at least about 0.3 percent zinc, for example, the ASTM designated magnesium-base alloy ZE10, which are usually cast at a temperature within the range of from about 1300° to 1350° F., columnar grains and so-called stringers, as defined below, tend to form in the outer portions commencing near the chilled surface and on in toward the center of the cast ingots or billets rather than equiaxed grains which are more desirable. Such columnar structure is particularly undesirable in castings intended for rolling in that it may cause the metal to crack severely when rolled. However, when equiaxed grains are present the rollability of the alloy is increased together with its strength potential.

The term "columnar grains" as used herein refers to a coarse structure of parallel columns of grains having the long axis perpendicular to the casting surface, whereas, the term "stringers" refers to a band at or near the casting surface comprising shorter columnar grains but, like the "columnar grains," not equiaxed in structure. Accordingly, the term "equiaxed grain" refers to a grain structure in a magnesium-base alloy wherein the axis of substantially all the grains is substantially the same length across any given cross section thereof.

Various methods have been and are presently practiced to obtain preferably a long lasting grain refinement effect in magnesium-base alloys such as, for example, by adding metallic elements to the alloy as nucleating agents such as, for example, zirconium, iron, aluminum, and carbon. The addition of such agents, however, to grain refine said ZE10 alloy in addition to being economically undesirable, has been found to be unsatisfactory in that by adding zirconium, for example, the cleanliness of the molten alloy deteriorates, that is, the number of oxide particles and flux inclusions increases in castings. The addition of iron on the other hand does not normally result in a lasting grain refinement at high alloying and casting temperatures. In addition, iron may create corrosion problems in the alloy. Furthermore, carbon treatments are not effective on alloys, such as ZE10, which do not contain aluminum. In view of the above difficulties, therefore, it would be highly desirable in the art to have a particular simple and economical process for grain refining zinc and misch metal-containing magnesium-base alloys, whereby a long lasting grain refinement effect may be obtained without the need of additional equipment or process steps.

The term "long-lasting grain refinement effect" as used herein means a grain refinement effect which persists throughout the period of settling, holding and casting without additional treatment in a large batch of the molten magnesium-base alloy specified herein to be grain refined in accordance with the present invention, for example, in batches containing 600 to 4000 pounds of molten metal.

An object of the present invention, therefore, is to provide a novel process for grain refining magnesium-base alloys containing zinc and rare earth metals.

Another object of the present invention is to provide a simple and economical method of imparting a lasting grain refinement to magnesium-base alloys containing up

2

to about 1.0 percent of rare earth metals and at least about 0.3 percent of zinc. A further object is to provide such a method for grain refining magnesium-base alloy ZE10 castings.

5 The appended two-figured lithograph, which will be discussed more fully hereinafter, of a photomicrograph taken at a 25X magnification of the magnesium-base alloy ZZE10 shows in FIGURE 1 the alloy when treated in accordance with the present invention and, as shown in FIGURE 2, when not so-treated, thus illustrating the fine equiaxed grain structure obtainable in said alloy when processed by the method of the present invention.

In general, the above and other objects and advantages have surprisingly been found obtainable, in accordance with the present invention, by casting or holding the magnesium-base alloy to be treated in the casting pot just prior to and during pouring at a temperature within the range of from about 1190° F. to about 1240° F., and preferably between 1220° F. and 1240° F. The time and other temperatures, such as those employed in melting, alloying, and settling the alloy prior to being cast, do not affect the grain refining, provided the aforesaid temperatures in the casting pot are observed just prior to and during pouring (casting) of the molten alloy. Higher temperatures than about 1240° F. should be avoided during casting, particularly when casting the ZE10 alloy. For example, the line carrying molten metal from the casting pot to the mold should not raise the temperature of the molten alloy above 1240° F.

30 The alloy to be treated, in addition to containing up to 1 percent rare earth metal, such as, for example, by the addition of misch metal (MM), and at least about 0.3 percent of zinc, should contain at least about 0.001 percent of iron. In most cases, however, such an iron content exists normally as an impurity in primary magnesium and ordinary magnesium alloys. Iron need not, therefore, normally be added to the alloy as a specific addition.

35 The method of the present invention, then, for grain refining a magnesium-base alloy as specified hereinbefore, comprises establishing a molten mass of said alloy at a temperature within the range of from about 1190° F. to about 1240° F. and, while maintaining said temperature, casting the metal into the desired configuration, 40 thereafter allowing the so-cast metal to solidify, thereby preparing fine grained cast articles. The present method has the advantages of simplicity and economy in that only the temperature of the molten metal need be controlled during the normal casting sequence, thus requiring no additional process steps or additional equipment.

45 The following examples serve to more fully illustrate the novel method of the present invention but are not intended to be construed as limiting it thereto.

50 *Example 1*

To show how columnar grains and stringers are eliminated and fine equiaxed grains produced for a lasting grain refinement effect various zinc and rare earth metal-containing magnesium-base alloys operable in the present novel process each having the composition indicated on Table I below were prepared in washed steel and clean graphite crucibles by melting, alloying and flux refining said alloys at 1400° F. using a crushed fused flux having a composition comprising 50 percent magnesium chloride, 25 percent potassium chloride, 20 percent barium chloride and 5 percent calcium fluoride. The melts were then held for the periods indicated in Table I, whereupon, each was sampled with a hot ladle while the melt was at a temperature within the range of from 1190° F. to 1400° F. for grain size determination and composition analysis. In the smaller melts (100 pounds), grain size

was estimated from the fractures obtained from 1½ inch diameter by 8 inch long bars which had been cast into a permanent steel mold (P.M.). Samples using a wedge mold were also obtained from the same region of the melt for spectrographic analysis. Melts prepared for direct-chill continuous casting (commonly referred to as solidification casting) were prepared in 600 pound batches and were also sampled for grain size and composition analysis. Other than the melts used for said direct-chill castings, which were cast in diameters as indicated in Table I, the grain size of which was determined metallographically, the grain size rating of the various melts was determined by visual comparison with the naked eye of the aforesaid fracture samples and standard samples. A rating number was given qualitatively related to the grain size and type was shown below:

| Equiaxed Number | Description of Grain Structure | Columnar Number |
|-----------------|--------------------------------|-----------------|
| .01             | Very fine                      | 1               |
| .02             | do                             | 2               |
| .03             | Medium                         | 3               |
| .04             | do                             | 4               |
| .05             | Very coarse                    | 5               |

The structure was rated with an equiaxed number only when there was a complete absence of columnar grains. If any columnar grains would appear the structure was rated with the respective columnar number.

For comparison purposes a portion of the melts prepared above as controls were processed and sampled in the same manner except that the casting temperatures employed were above 1240° F. The pertinent data and results for these controls is also indicated in Table I.

external vertical wall of the cylindrical cavity caused the metal to freeze by spraying water on the mold wall as the pouring continued and the resulting solidifying billet moved downward.

5 Part of the billet so formed was then cut into 2 inch slices and a representative sample slice selected for a grain sized and structure determination. The selected sample was then transversely cut into quarters and one of the quarters cut into 4 segments perpendicularly to the transverse cut. Said segments were designated 1 through 4 toward the center of the billet, and a portion of each segment was prepared for metallographic examination. A photomicrograph of the polished portions was taken and is shown as FIGURE 1 on the appended lithograph.

10 15 For comparison, the above procedure was duplicated in every respect again using the ZE10 alloy except that the casting was done at a temperature above 1240° F., namely, at 1300° F. The photomicrographs obtained from the samples derived from this casting are shown as FIGURE 2 of the appended lithograph.

15 An examination of the grain structure of the segment portion designated number 1 in each figure clearly shows the absence of stringers and columnar grains in the outer portions (close to the chilled surface) of the casting of

20 FIGURE 1 cast in accordance with the present invention as compared to the pronounced presence of same near the surface of the ZE10 alloy of FIGURE 2, which was not cast in accordance with the present invention. It should also be noted in segments 2 through 4 (which proceed to the center of the casting) that the size of the equiaxed grains in FIGURE 1 is markedly finer than that of the alloy of FIGURE 2, illustrating the exceptionally fine equiaxed grains obtainable by the method of the present invention.

30 35 It is manifest that various modifications can be made

#### TYPE I

| Sample | Size of Melt (Lb.) | Type of Cast                    | Holding History |                  | Casting Temp., ° F. | Grain Structure |                        | Composition, Percent <sup>1</sup> |      |      |                 |      |
|--------|--------------------|---------------------------------|-----------------|------------------|---------------------|-----------------|------------------------|-----------------------------------|------|------|-----------------|------|
|        |                    |                                 | Time, Hrs.      | Temp., ° F.      |                     | Grain Rating    | Width of Stringer Band | Al                                | Fe   | Mn   | MM <sup>2</sup> | Zn   |
| 1..... | 600 (control)      | 9" dia. D.C. <sup>3</sup>       | { 18<br>2       | { 1,300<br>1,205 | 1,300               | .04             | 1" wide                | .003                              | .030 | .08  | .18             | 1.36 |
| 2..... | 600.....           | 9" dia. D.C. <sup>3</sup>       | { 18<br>2       | { 1,330<br>1,295 | 1,230               | .03             | None                   | .006                              | .021 | .07  | .19             | 1.31 |
| 3..... | 600 (control)      | 12" dia. D.C.                   | 18              | 1,300            | 1,300               | .12             | 1½" wide               | .003                              | .035 | .03  | .09             | 1.37 |
| 4..... | 600.....           | 12" dia. D.C.                   | 14              | 1,300            | 1,237               | .03             | None                   | .002                              | .028 | .006 | .09             | 1.45 |
| 5..... | 100 (control)      | 1½" dia. X 10 P.M. <sup>4</sup> | 16              | 1,350            | 1,300               | 3.0             | do                     | .016                              | .037 | .072 | .16             | 1.43 |
| 6..... | 100.....           | 1½" dia. X 10 P.M. <sup>4</sup> | 17              | 1,350            | 1,220               | .01             | do                     | .018                              | .029 | .071 | .17             | 1.46 |
| 7..... | 100 (control)      | 1½" dia. X 10 P.M.              | 4               | 1,300            | 1,300               | 4.0             | do                     | .006                              | .029 | .01  | .19             | 1.34 |
| 8..... | 100.....           | 1½" dia. X 10 P.M.              | 6               | 1,300            | 1,220               | .01             | do                     | .005                              | .026 | .01  | .18             | 1.34 |

<sup>1</sup> Balance essentially of magnesium. <sup>2</sup> MM = misch metal. <sup>3</sup> D.C. = direct chilled. <sup>4</sup> P.M. = permanent mold.

#### Example II

To illustrate application of the grain-refining method of the present invention with respect specifically to direct-chill casting, a well known casting technique, of the magnesium-based alloy ZE10 which has the nominal composition of 1.3 percent zinc, 0.2 percent misch metal (MM), and 0.002 percent iron, the balance being essentially magnesium, about 600 pounds of the alloy was melted under a protective cover of the flux hereinbefore used and defined, whereupon it was continuously cast using a direct-chill mold to produce a 12 inch diameter billet 120 inches in length. The direct-chilled mold comprised an open-topped cylindrical cavity 12 inches in diameter having a hydraulically downwardly moving bottom part. The melt of ZE10 alloy while at a temperature within the range of from 1220° F. to 1240° F. was continuously poured into said cavity, whereupon, after a solidified head of metal had formed against the mold bottom, said bottom was concurrently and continuously moved downward as the melt was being poured into the mold. Water pipes located annularly around the

55 in the process of the present invention without departing from the spirit or scope thereof and it is understood that I limit myself only as defined by the appended claims. I claim:

1. A method of grain refining a magnesium-base alloy 60 containing rare earth metals and zinc which comprises, establishing a molten mass of the alloy to be grain refined, casting said molten mass from a temperature within the range of from about 1190° F. to about 1240° F., thereby imparting to the cast alloy a fine equiaxed grain structure, and cooling to solidify it.

2. The method of claim 1 wherein the casting temperature is within the range of from about 1220° F. to about 1240° F.

3. The method of claim 1 wherein the magnesium-base alloy to be grain refined contains at least about 0.001 percent by weight of iron.

4. The method of claim 1 wherein the magnesium-base alloy to be grain refined contains by weight up to about 1 percent of rare earth metals and at least about 0.3 percent of zinc.

5. The method of claim 1 wherein the magnesium-base alloy to be grain refined is the ASTM designated ZE10 alloy.

6. A method of grain refining a magnesium-base alloy containing up to about 1.0 percent of misch metal and at least about 0.3 percent of zinc and at least about 0.001 percent of iron which comprises, establishing a molten mass of the alloy to be grain refined, casting said molten mass from a temperature within the range of from about 1190° F. to about 1240° F., thereby imparting to the cast alloy a structure consisting of fine equiaxed grains, and solidifying the so-cast alloy by allowing it to cool.

7. The method of claim 6 wherein the casting temperature is within the range of from about 1220° F. to 1240° F.

8. A method of imparting a lasting fine equiaxed grain structure to a direct-chilled magnesium-base alloy casting of ZE10 which comprises, establishing a molten mass of said ZE10 alloy, continuously casting and solidifying the molten alloy into a directly chilled mold from a temperature within the range of from about 1190° F. to about 1240° F., thereby to continuously produce a solidified casting of said ZE10 alloy having a lasting fine equiaxed grain structure throughout.

9. A method of eliminating columnar and stringer type grain structure in magnesium-base alloy castings containing by weight up to about 1.0 percent of misch metal and at least about 0.3 percent of zinc and 0.001 percent of iron which comprises, casting the molten alloy by a continuous solidification process from a temperature within the range of from about 1190° F. to about 1240° F., thereby to produce a casting of said alloy essentially free of columnar and stringer type grains.

#### References Cited by the Examiner

##### FOREIGN PATENTS

359,425 10/1931 Great Britain.

##### OTHER REFERENCES

Magnesium: 1st Ed., American Magnesium Corporation, 1923, TN 799 M2 A6, page 115.

Magnesium: American Society for Metals, 1946, TN 799 M2 M18, page 73.

Journal of Metals: "The Properties of Sand Cast Magnesium-Rare Earth Alloys," 1949, pp. 968-971.

J. SPENCER OVERHOLSER, Primary Examiner.

R. S. ANNEAR, Assistant Examiner.